

## UNITED STATES PATENT OFFICE

CAMILLE DREYFUS, OF NEW YORK, N. Y.

## PILE FABRIC

No Drawing.

Application filed November 3, 1928. Serial No. 317,126.

This invention relates to the preparation of pile fabrics having yarns of natural silk and yarns of artificial filaments containing organic esters of cellulose.

5 An object of my invention is to produce pile fabrics having both yarns of natural silk and yarns of organic esters of cellulose therein, wherein the 'yarns of the organic esters of cellulose have a natural luster or 10 sheen. Objects of my invention will appear from the following detailed description.

In the ordinary textile operations involving the manufacture of fabrics containing natural silk, the practice is to weave the 15 silk yarn while it still has the gum therein in order that the silk may have sufficient strength to withstand the drastic strains due to textile operations. I have found, however, that if silk, while in the gum, is woven 20 with yarn containing organic derivatives of cellulose, after the fabric is finished, the yarns of the organic derivatives of cellulose lose some of their luster and sheen in the process of boiling off the fabric to remove 25 the gum from the natural silk even if the degumming of the silk is carried out at comparatively low temperatures, say for instance, 80° C. Since pile fabric such as 30 velvet depends so much for its beauty on the sheen of the yarn, if a mixed fabric containing natural silk and organic ester of cellulose yarn were made in this manner, the luster of the same would become so subdued by the boiling off process that its effect 35 would be materially reduced. I have found that if natural silk yarn is first degummed to an appropriate extent and then woven into pile fabric, a product is produced that has a beautiful luster and sheen after the 40 dyeing and finishing operations have been accomplished.

In accordance with my invention I prepare a pile fabric from yarns of organic esters of cellulose that are apt to become 45 delustered when boiled with water or aqueous liquids and natural silk yarn from which the gum has been previously removed to the extent required for the particular case. The organic esters of cellulose employed for making the yarn to be used in

my invention may be any suitable ones such as cellulose acetate, cellulose formate, cellulose propionate and cellulose butyrate. These yarns may be associated with yarns of other materials such as cotton, wool or 55 flax. As stated the silk yarn to be used is first degummed to the desired extent prior to weaving.

The organic ester of cellulose yarn and the so degummed natural silk yarn are then 60 woven into any suitable pile fabric such as transparent velvet, printed velvet or heavier velvet. The fabric may be constructed so that the back thereof is entirely or mostly 65 of natural silk while the pile is composed entirely of yarn made of cellulose acetate. If desired the pile may be made wholly of natural silk while the back is made of cellulose acetate yarn. Likewise the back may 70 be made entirely of natural silk and the pile of mixed natural silk and cellulose acetate 75 yarn or vice versa. Yarns of other materials such as cotton or reconstituted cellulose (artificial silk) may also be used either in the back or in the pile or both.

Since the fabric made in accordance with my invention does not have to be subjected to a degumming or boiling off treatment to remove the gum from the silk, there is no 80 danger of the yarns of the organic esters of cellulose becoming delustered. By my process, therefore, a finished pile fabric of the natural beautiful sheen or luster of organic esters of cellulose yarn is produced. From the point of view of economy, my process is 85 of great advantage since the natural silk may be degummed as above at higher temperatures and in much less time.

The pile fabric made by my invention may be subjected to any desired finishing treatment such as dyeing, scouring, printing, etc. 90 as is well understood in the art.

It is to be understood that the foregoing detailed description is given merely by way of illustration and that many variations may be made therein without departing from the 95 spirit of this invention.

Having described my invention what I claim and desire to secure by Letters Patent is:

1. Method of making pile fabric containing natural silk and yarns of organic esters of cellulose that is apt to become delustered when exposed to boiling water comprising degumming undyed natural silk to the desired extent and then weaving the undyed degummed silk together with said organic ester of cellulose yarn in such a manner as to form a pile fabric which need not be subjected to a degumming process, whereby finished fabric having the natural sheen or luster of the organic ester of cellulose yarn may be produced.
2. Method of making pile fabric containing natural silk and yarns of cellulose acetate that is apt to become delustered when exposed to boiling water comprising degumming undyed natural silk to the desired extent and then weaving the undyed degummed silk together with said cellulose acetate yarn in such a manner as to form a pile fabric which need not be subjected to a degumming process, whereby finished fabric having the natural sheen or luster of the cellulose acetate yarn may be produced.

In testimony whereof, I have hereunto subscribed my name.

CAMILLE DREYFUS.